

## UNITED STATES PATENT OFFICE

2,000,411

## TREATMENT OF HYDROCARBON OILS

Jacque C. Morrell and Gustav Egloff, Chicago,  
Ill., assignors to Universal Oil Products Com-  
pany, Chicago, Ill., a corporation of South  
Dakota

No Drawing. Application December 30, 1931,  
Serial No. 583,916

## 4 Claims. (Cl. 44—9)

This invention relates to the treatment of hydrocarbon oils and refers more particularly to the treatment of low boiling distillates produced in the cracking of heavier higher-boiling fractions.

More specifically, the invention has reference to a process for treating hydrocarbon mixtures undergoing decomposition and conversion reactions or the lower boiling vaporous products of these reactions to produce substantial amounts of compounds which add materially to the anti-knock value of the gasoline finally produced from the process.

While the cracking process as at present generally practiced in the petroleum industry tends to the production of gasolines having anti-knock characteristics superior to those possessed by corresponding gasoline fractions produced by the straight run distillation of crude petroleums, it may frequently happen that the production of a cracked gasoline of a knock rating rendering it saleable as a premium motor fuel may entail the use of relatively severe cracking conditions with attendant increased losses in fixed gases and coke and a decrease in the overall yield of the desired product. In the majority of cases for any given stock charged to the cracking process, there exists an optimum set of conditions for producing a maximum yield of gasoline of good anti-knock value, the use of more severe conditions, while they may produce gasoline boiling range fractions closely approximating a mixture of aromatic hydrocarbons in composition, producing not only excessive gas losses but a very material lowering in yield of gasoline so that in this respect it may be stated that the production of increased yields of anti-knock gasoline by the cracking process is limited by economic considerations.

The present invention has as one of its objects provision of a process by which the economic disadvantages of producing high anti-knock value gasoline by cracking may be offset by the production concurrently in the cracking process of compounds having a specially high anti-knock value so that the product of the operation considered as a whole is of the high quality desired and the necessary yields are maintained.

In one specific embodiment the invention comprises treating cracked hydrocarbon vapors with halogenated or sulfonated hydrocarbons and sodamide for the production of amines to increase the anti-knock value of the gasoline and other treating effects.

The types of hydrocarbon derivatives which it

is preferred to use are preferably of the aromatic series such as chlorine derivatives of benzol, toluol, xylol, etc., or their corresponding sulphonate or sulphonic acids. The reaction of such derivatives with sodamide ( $\text{NaNH}_2$ ) results in general in the combination of the sodium with the hydrogen-substituting group in the hydrocarbon and the substitution of the amino or  $\text{NH}_2$  group therein to produce corresponding amines. The general reaction may be typified by the following equation:



in which R represents any monovalent hydrocarbon radical, either of the alkyl or aryl groups. Similarly the chlorine atom in the above equation may be substituted by the sulphonate or sulphonic groups according to the equations following:



Sodamide is a compound well known in the arts and is used extensively in the manufacture of dyes and in other chemical processes. It is usually manufactured by conducting dry ammonia gas into molten sodium or by dissolving sodium in liquid ammonia. Other methods less commonly used consist in treating sodium oxide with ammonia or by treating sodium hydride with ammonia. Amides strictly analogous to that of sodium have been prepared from each of the other metals of the alkali group, that is, potassium, lithium, rubidium and caesium by the same general methods but none are of great commercial importance on account of the higher cost of the base materials and in that they offer no decided advantages over the sodium compound in most instances. The sodium compound melts at approximately  $310^\circ \text{ F.}$  and boils at  $750^\circ \text{ F.}$  It will be evident from its constitution that it provides a powerful reagent for use in many chemical processes, particularly those in which a reducing action is required or when it is necessary to introduce sodium into the sphere of reaction.

Several alternative methods of operation are possible and are comprised within the scope of the invention. As a general rule, the conditions under which the general reactions are brought about correspond to those of cracked vapors undergoing fractionation under super-atmospheric pressure following the reaction zone of a cracking process, these conditions involving temperatures of from approximately  $300$  to  $600^\circ \text{ F.}$

and pressures in the approximate range of 100 to 400 pounds per square inch. According to one method of operation the vapors entering a primary fractionator or separator may receive increments respectively of chlorinated or sulphonated hydrocarbons and at approximately the same point the proper amount of sodamide, the subsequent fractionation serving to remove the sodium salts produced incidentally to the main reaction as a fused or soluble mass in the bottom of the fractionator or separator, and the production of amines which distill over with the gasoline fractions and add to their anti-knock value.

Another possible method of operation which may, however, require more precautions as to exact control of operation, may consist in either passing the cracked vapors after the addition of the halogenated or sulphonated hydrocarbon derivatives through a stationary body of molten sodamide or upwardly countercurrent to a down-flowing stream in suitably designed apparatus.

The effect on the anti-knock value of gasoline of certain aromatic amines which may be produced in the gasoline fractions from a cracking process according to the present invention is shown by the following table in which the effect on anti-knock value is measured by the percentage increase in the "H. U. C. R." (highest useful compression ratio). It will be observed that the greatest effect is produced by methyl aniline and xylidine though their effects are only slightly above that of aniline as the simplest member of the series and which would result from the interaction of chlorbenzol and sodamide.

35

#### Percentage increase of H. U. C. R.

With No. 1 petrol obtained by addition of 5% by volume of common organic substances selected with reference to solubility and boiling point

| 40 | Name of substance  | Chemical formula | Melting point °C. | Boiling point °C. | Critical point °C. | Effect on H. U. C. R. | 40 |
|----|--------------------|------------------|-------------------|-------------------|--------------------|-----------------------|----|
|    | Aniline.           | $C_6H_5N$        | -5                | 184               | 433 dry            | +21.7                 |    |
|    | Methyl aniline.    | $C_6H_5NH_3$     | -57               | 194               | 432-442            | +22.2                 |    |
|    | Ethyl aniline.     | $C_6H_5NH_2$     | -63               | 204               | 425-415            | +10.4                 |    |
|    | Di-methyl aniline. | $C_6H_3(NH_3)_2$ | +2                | 195               | 420-400            | +1.7                  |    |
| 45 | Di-ethyl aniline.  | $C_6H_3(NH_2)_2$ | -38               | 216               | 411-300            | 0                     | 45 |
|    | Benzyl aniline.    | $C_6H_5CH_2NH_2$ | +33               | 310               | Decomp. 470        | +0.5                  |    |
|    | Toluidine.         | $C_6H_5NH_2$     | -21               | 200               | 430-441            | +18.3                 |    |
|    | Xylidine (M).      | $C_6H_3(NH_2)_2$ | +49               | 215               | 448                | +22.8                 |    |

It is contemplated to use mixtures of hydrocarbon derivatives which are adaptable to use in the process, for example, light coal tar distillates may be chlorinated and introduced into the cracking vapors along with sodamide as already described without resorting to the usually tedious methods of separation or individual hydrocarbons by fractionation.

The particular hydrocarbon derivative or mixture of such employed in the process and the amount used will depend upon a variety of factors such as the cost of the compound or mixture, the character of the cracked products (which in turn depends upon the character of the charging stock and the conditions of operation) and the knock rating desired in the finished gasoline. Chlorbenzol is of general application, as the aniline which results from it by reaction with sodamide has a high effect on the anti-knock value of a given gasoline, this being only slightly exceeded by such compounds as cumidine, xylidine, monomethylaniline, toluidine, etc., as shown by the table.

In addition to the production of amines which add to the anti-knock value of the gasoline, other treating effects may be produced by the use of sodamide if this is used in excess over that re-

quired for interaction with the hydrocarbon derivative employed. It has at times a very pronounced desulphurizing action on account of the great affinity of the sodium for sulphur in such compounds as mercaptans, sulphur ethers, etc., and may result in substantial sulphur reduction in the finished product depending upon the types of sulphur compounds present in the cracked vapors and other conditions of operation as well as the excess of sodamide used.

The process of the invention may be used as a single treatment on cracked vapors or in combination with preceding or succeeding treatments for producing as an overall result a finished product of desired characteristics. For example, the vapors may be treated by special desulphurizing and/or polymerizing steps prior to the introduction of the reactants for the production of amines and still further vapor phase treatments, suitable settling periods or filtering by inert or absorbent materials may follow. In the majority of instances a final rectification to produce an end point gasoline is preferable. Furthermore, the condensed product may require a light final washing to remove traces of reaction products.

As an example of a treatment which may be conducted according to the process of the invention and the results obtainable therefrom, the cracked vapors of approximate gasoline boiling point range coming from the fractionator of a cracking process operating on Mid-Continent residuum may be considered. Such vapors may be evolved from the fractionator under a pressure of approximately 20 pounds per square

10

15

20

25

30

35

inch and a temperature of 500° F. Chlorbenzol may be injected into these vapors at the rate of about 12 pounds per barrel of final distillate along with approximately 4½ pounds of sodamide, the vapors then passing to settling and filtering equipment to remove sludge mixtures and salts produced by the reaction. The gasoline produced by fractionating and contacting these vapors with solid absorbent materials without the use of chlorbenzol and sodamide upon the vapors according to the process of the invention may have the properties shown in the "untreated" column following, while gasoline produced by applying the process of the invention may have the properties shown in the "treated" column.

|                                                                         | Untreated | Treated | 65 |
|-------------------------------------------------------------------------|-----------|---------|----|
| Octane number.                                                          | 66        | 83      |    |
| Color, Saybolt.                                                         | 11        | 30      |    |
| Gum content by copper dish.                                             | 275       | 25 mg.  |    |
| Sulphur content.                                                        | 0.22      | 0.06    |    |
| Color stability or loss in Saybolt degrees in the 4-hour sunlight test. | 10        | 3-4     | 70 |

The yield of gasoline in both cases may be approximately 60% of the residuum processed, with the maximum cracking temperature em-

5

10

15

20

25

30

65

70

75

ployed 930° F. with a pressure of 250 pounds per square inch. To produce the 82 octane number by straight cracking and fractionation without the addition of a special treating reagent according to the process of the invention it may entail a reduction in yield to approximately 50%, which is a serious consideration in commercial work and which might render the process uneconomical. Thus the application of the present invention is shown to have a definite commercial value.

The foregoing general description of the process of the invention and the example of the results obtainable by one operation thereof is sufficient to enable one skilled in the art to recognize its value, but since the exact type of operation may be considerably varied and the amounts of reagents also varied in the treatment of different stocks, the process as disclosed is not to be construed in any way as a limitation upon the broad scope of the invention.

We claim as our invention:

1. The method of improving the overhead product of a distillatory gasoline-producing system, which comprises introducing a sulphonating agent to a vapor zone of said system to form a sulphonated hydrocarbon derivative, contacting the vapors containing said derivative with sodamide, and condensing the thus treated vapors.

2. The method of improving the overhead

product of a distillatory gasoline-producing system, which comprises introducing a sulphonated hydrocarbon derivative to a vapor zone of said system, contacting the vapors containing said derivative with sodamide, and condensing the thus treated vapors.

3. In a process for improving the anti-knock characteristics of the overhead distillate product resulting from the conversion of higher boiling hydrocarbons into relatively lower boiling hydrocarbons by the cracking process the improvement which comprises introducing into the vapor zone of the said cracking process a sulphonating agent to produce a sulphonated hydrocarbon derivative, and thereafter subjecting the mixture of hydrocarbons and the aforementioned derivative to contact with sodamide, and condensing the thus treated vapors.

4. In a process for improving the antiknock characteristics of the overhead distillate product resulting from the conversion of higher boiling hydrocarbons into relatively lower boiling hydrocarbons by the cracking process, the improvement which comprises introducing into the vapor zone of the said cracking process a sulphonated hydrocarbon derivative and thereafter subjecting the mixture of hydrocarbons and the aforementioned derivative to contact with sodamide, and condensing the thus treated vapors.

JACQUE C. MORRELL. 30  
GUSTAV EGLOFF.